

3,188,164  
**POLYPROPYLENE FIBERS DYED WITH  
 4-NITROACRIDONE DYES**

Joseph W. Dehn, Jr., Great Neck, and Harold J. Kuhefuss, Brooklyn, N.Y., and John J. Maitner, Hazlet, N.J., and Anthony J. Salina, New York, N.Y., assignors to Interchemical Corporation, New York, N.Y., a corporation of Ohio  
 No Drawing. Filed Jan. 22, 1963, Ser. No. 253,040  
 6 Claims. (Cl. 8—55)

This invention relates to polypropylene fibers dyed with 4-nitroacridone dyes.

It has been found that 4-nitroacridone and some of its derivatives act as disperse dyes for polypropylene fibers when applied by more or less conventional means. The dyes display much better lightfastness when dyed on polypropylene fibers than do the commercially available dyes recommended by the fiber manufacturers.

The detailed procedure that follows illustrates a specific embodiment of this invention.

### EXAMPLE

A mixture of 3.00 g. of the dye, 1.00 g. of Marasperse N, and 1.00 g. of Cyclopone AF was combined with water and ground with a hand muller to disperse the dye. After the material was oven dried, it was ground to a powder with mortar and pestle and used to make up the dyebath. A convenient weight of polypropylene fiber in the form of cloth was scoured 30 minutes at 70° C. in an aqueous solution of 1% (based on fiber weight) of an anionic wetting agent such as Sulframin AB and 0.25% (based on fiber weight) of sodium carbonate. A dyebath was made up having about 40 times the weight of the fiber. The dyebath was simply water containing 1% (based on fiber weight) of an anionic wetting agent such as Sulframin AB and ½% (based on fiber weight) of the dye. The cloth was entered at room temperature and the dyebath was heated at about 100° C. for about 2 hours. To remove surface dye, the goods were then soaped 30 minutes at 70° C. in an aqueous solution of about 2% sodium carbonate (based on fiber weight) and about 1% (based on fiber weight) of a suitable dispersing agent such as Sulframin AB. The goods were then rinsed and dried.

Another set of dyeings was made using a similar procedure but with 2% dyestuff instead of ½%.

The table below gives specific examples, showing the dyestuff used, its color on polypropylene fiber, and the lightfastness.

### Dyed polypropylene fiber

| Dyestuff                                 | Color  | Light fastness                                                                                                      |
|------------------------------------------|--------|---------------------------------------------------------------------------------------------------------------------|
| 4-nitroacridone                          | Yellow | No break at 80 hours.                                                                                               |
| 2-methoxy-4-nitroacridone                | Orange | Noticeable break at 80 hours.                                                                                       |
| 5-methoxy-4-nitroacridone                | do     | Noticeable break at 40 hours.                                                                                       |
| 7-methoxy-4-nitroacridone                | Pink   | No break at 80 hours.                                                                                               |
| 2, 5-dimethoxy-4-nitroacridone           | Orange | Very slight break at 40 hours; slight break at 80 hours.                                                            |
| 2, 7-dimethoxy-4-nitroacridone           | Mauve  | Very slight break at 20 hours; slight break at 40 hours; no additional break at 60 hours; slight break at 80 hours. |
| 5, 7-dimethoxy-4-nitroacridone           | Pink   | Slight break at 80 hours.                                                                                           |
| 5, 8-dimethoxy-4-nitroacridone           | do     | Distinct break at 20 hours.                                                                                         |
| 6, 7-(or 7, 8)-dimethoxy-4-nitroacridone | do     | Very slight break at 40 hours; slight break at 80 hours.                                                            |
| 1-chloro-4-nitroacridone                 | Orange | Very slight break at 20 hours; slight break at 40 hours; distinct break at 60 hours.                                |
| 2-chloro-4-nitroacridone                 | do     | Slight break at 40 hours; noticeable break at 80 hours.                                                             |
| 2-bromo-4-nitroacridone                  | do     | Slight break at 40 hours; another slight break at 60 hours; another slight break at 80 hours.                       |
| 7-bromo-4-nitroacridone                  | Yellow | Slight break at 60 hours; noticeable break at 80 hours.                                                             |
| 7-methyl-4-nitroacridone                 | do     | Very slight break at 40 hours; slight break at 60 hours; another slight break at 80 hours.                          |
| 5-methylthio-4-nitroacridone             | do     | Very slight break at 20 hours; slight break at 40 hours; another slight break at 60 hours.                          |

The test pieces were all examined at 20-hour intervals up to 80 hours. Changes were noted, at least until a distinct break occurred. Lightfastness tests were made in the conventional way on the Fade-O-Meter.

The preparation of the dimethoxy-4-nitroacridone dyes is described in application Serial No. 152,670, filed November 15, 1961. The preparation of 5-methylthio-4-nitroacridone (5-methylmercapto-4-nitroacridone) is described in application Serial No. 237,394, filed November 13, 1962.

Marasperse N is a ligno sulfonate.

Cyclopone AF is sodium N-acyl-N-methyl-taurate.

Sulframin AB is sodium alkyl-benzene-sulfonate.

What is claimed is:

1. Polypropylene fiber dyed with a 4-nitroacridone dye selected from the group consisting of

(a) a compound having the formula



20

wherein R is selected from the group consisting of H and CH3O, at least one R being H,

(b) a compound having the formula



25

wherein R is selected from the group consisting of H, Cl, and Br, two of the R's being H,

(c) a compound having the formula



30

wherein one R is H and the other R is CH3O,

(d) 7-methyl-4-nitroacridone, and

(e) 5-methylthio-4-nitroacridone.

35

40

45

3

2. Polypropylene fiber dyed with a dye having the formula



wherein R is selected from the group consisting of H and CH<sub>3</sub>O, at least one R being H.

3. Polypropylene fiber dyed with a dye having the formula



wherein R is selected from the group consisting of H, Cl, and Br, two of the R's being H.

4

4. Polypropylene fiber dyed with a dye having the formula



10 wherein R is H and the other R is CH<sub>3</sub>O.

5. Polypropylene fiber dyed with 7-methyl-4-nitroacridone.

6. Polypropylene fiber dyed with 5-methylthio-4-nitroacridone.

15

References Cited by the Examiner

UNITED STATES PATENTS

- |    |           |      |                 |           |
|----|-----------|------|-----------------|-----------|
| 20 | 2,005,303 | 6/35 | Spiegler et al. | 260—279 X |
|    | 3,054,793 | 9/62 | Howard et al.   | 260—279 X |
|    | 3,074,950 | 1/63 | Deutsche et al. | 260—279   |

NORMAN G. TORCHIN, Primary Examiner.